# EUROPEAN PATENT SPECIFICATION

(11) **EP 0 064 863 B1**
(45) Date of publication and mention of the grant of the patent: **09.07.1986**
(21) Application number: 82302299.1
(22) Date of filing: 05.05.1982
(51) Int. Cl.: C21C 5/44, F27D 1/16, B22D 11/10

(54) **Monolithic refractory layer for metallurgical vessels and method of application**
Monolithische feuerfeste Schicht für metallurgische Gefässe und Anwendungsverfahren
Couche monolithique et réfractaire pour récipients métallurgiques et méthode d'utilisation

(30) Priority: 08.05.1981 JP 68940/81
(43) Date of publication of application: 17.11.1982
(73) Proprietor: QUIGLEY COMPANY INC., New York, N.Y. 10017 (US)
(72) Inventor: Asaka, Eiji, Ichihara-shi Chiba Pref. 290 (JP); Ishikawa, Kentaro, Ohta-Ku Tokyo 144 (JP); Kawai, Ryozo, Taito-ku Tokyo 111 (JP); Taniguchi, Teruhiko, Kobe-Shi Hyogo Pref. 655 (JP)
(74) Representative: Graham, Philip Colin Christison

## Description

This invention relates to a novel refractory layer for metallurgical vessels, particularly the protective layer for a tundish, and a method of application of the layer within such vessels.

In the continuous casting of steel, molten steel is transferred by means of a ladle from the steelmaking vessel to a tundish, from which it is constantly fed into casting molds. Such continuous feeding is accomplished by maintaining a reservoir of the molten steel within a tundish lined with such as refractory brick and having from one to five nozzles located on the tundish bottom. The tundish is customarily heated to about 1000 to 1300°C before being placed into service to minimize the tendency of the molten steel to cool and solidify during the pouring, with resultant nozzle clogging and adhesion of the solidified steel to the lining. Upon completion of a pouring, any slag or solidified steel retained in the tundish is scraped from the lining, and the eroded areas of the lining are repaired. Since the lining is readily attacked by molten steel and slag, frequent relining of the tundish is required, resulting in a considerable expenditure of time, labor and refractory material.

To extend the effective life of a tundish lining, current practice is to cover the lining with a protective layer, using either a trowelling material or lagging sheets. This protective layer should adhere well to the working lining and be strong as well as impermeable to molten steel and slag. The layer should also have a tendency to separate immediately behind any slag or solidified steel retained in the tundish at the completion of a pouring to permit the ready removal of the slag or solidified steel without damage to the lining; this tendency is commonly referred to as distintegrat- ability.

Trowelling materials used for the protective layer are generally of magnesia, alumina or alumina-silica based refractory aggregate. The material is simply slurried in water and trowelled onto the surface of the tundish lining. Such an operation, however, requires considerable time, skill and labor. In addition, the resulting protective layer contains a considerable amount of water and has poor insulating properties. A tundish having such a protective layer must, as in the case of a tundish with only a refractory lining, be preheated for from two to five hours until its temperature is about 1000 to 1300°C prior to use. Such heating is undesirable from the standpoint of energy conservation.

The lagging sheet, which is also referred to as insulation panel or tundish board, is generally prepared from a slurry of refractory aggregate, fibrous material and thermosetting resin in water or other liquid. The slurry is drained of excess liquid and formed into a sheet, and the sheet is then oven dried to cure the resin. The lagging is installed over the refractory lining, the seams between adjacent sheets being filled with a combination of mortar plus a strip of the lagging material attached to the seams and fixed with nails. Since the lagging has good insulating properties and normally need be heated to a temperature of only about 500°C before being placed into service, considerable energy savings over the trowelling method is realized. But the installation of the lagging is difficult and time consuming, and the lagging is easily eroded, particularly at the seams.

It is known from GB-A-1434662 to apply a refractory layer within a metallurgical vessel by positioning a former within the vessel, introducing a quartzite-based material into the space between the former and the vessel, which material contains from 0.5 to 1.5% by weight of a thermosetting resin and optionally a fluxing agent such as boric oxide, pre-heating the material at 100-280°C, removing the former and then heating at a higher temperature, e.g. 1100°C. It is also known from DE-A-2824773 to use a resin- coated refractory material including also fibrous material, magnesia and inorganic binder to form such a refractory layer and to use pressurised gas to introduce the material between the vessel and a former.

It is a primary object of the present invention to provide a refractory layer for a metallurgical vessel, particularly the protective layer of a tundish, and a method for its application which overcomes the drawbacks of existing techniques.

Accordingly, the present invention provides a method of applying a monolithic refractory layer within a metallurgical vessel, which comprises positioning within the vessel a mold having an outer surface substantially conforming to the configuration of the inner surface of the vessel so as to provide a substantially uniform space between the mold outer surface and the vessel inner surface; filling the space with a substantially dry particulate mixture comprising at least about 70 weight percent refractory aggregate, from about 0.5 to 20 weight percent thermosetting resin and from about 0.5 to 10 weight percent inorganic binder; heating the mixture to cure the resin; and removing the mold; characterised in that either said binder has water of crystallisation or said mixture comprises about 0.5 to 10 weight percent of a particulate inorganic compound having water of crystallisation in addition to said binder.

In preferred embodiments of the invention, the resin is coated on the refractory aggregate and the refractory aggregate has a maximum particle size of about 5 millimetres. The mixture may additionally comprise up to about 10 weight percent fiber having a length of preferably from about 5 to 15 millimeters. Preferably, the refractory is deadburned magnesia, while the resin is a phenol-formaldehyde resin and is cured at a temperature of from about 150 to 250°C. The mixture is conveniently introduced to fill the space with the aid of pressurized gas, the layer preferably being the protective layer of a tundish and having a thickness of from about 10 to 50 millimeters.

The present invention further provides for a metallurgical vessel which comprises a monolithic layer of a resin-bonded particulate refractory aggregate applied by the method of the invention.

The novel features and advantages of the present invention will become apparent from a reading of the following description in conjunction with the accompanying drawing of a preferred embodiment.

The drawing is a pictorial representation of a preferred method of applying a monolithic refractory protective layer on the working lining of a tundish using pressurized air to aid in applying the layer.

To apply a protective layer by this preferred method to a tundish 10, which comprises a steel shell 12 with a working lining 14 of such as refractory brick or a castable, a mold 16 fabricated from mild steel plate and having its outer surface 18 substantially conforming to the inner surface 20 of tundish 10 is used.

Mold 16 is placed within tundish 10 as shown so as to provide a substantially uniform space 22 between mold outer surface 18 and tundish inner surface 20. Space 22 may be from about 5 to 100 millimeters, but will normally be from about 10 to 50 millimeters. While substantially uniform, space 22 may be slightly greater in areas of extreme wear, such as the region of tundish 10 into which molten steel is poured from a ladle. For example, space 22 may be substantially 30 millimeters, but as much as 50 to 60 millimeters in high wear areas.

Mold 16 is equipped with air vents 24 and a heating element, either electrical or gas fired, not shown. Mold 16 is also provided with an inlet pipe 26, which is equipped with an automatic valve 28 and is connected to one end of a hose 30. The other end of hose 30 is connected through a valve 32 to the bottom of a supply tank 34 containing a dry particulate refractory mix 36. Supply tank 34 is connected through valves 38 and 40 to an air container 42, which in turn is connected to a source of compressed air, not shown. Air container 42 is also connected through valve 44 to hose 30 just downstream of valve 32.

Before the protective layer is to be formed, tundish inner surface 20 and/or mold 16 are preferably heated to from about 150 to 250°C. Valves 38, 40 are opened to supply air pressure to supply tank 34. Then automatic valve 28 and valve 32, and at the same time valve 44, are opened to release a mixture of refractory mix 36 from supply tank 34 and compressed air from air container 42 through hose 30 into space 22. As soon as space 22 is filled with refractory mix 36, the filling normally requiring a period of less than five minutes, automatic valve 28 closes. Mold 16 is then heated to or, if previously preheated, held at 100 to 300°C, preferably 150 to 250°C, to cure the resin content of refractory mix 36 in space 22. Mold 16 is then removed to leave on working lining 14 a layer of seamless monolithic refractory which has a thickness substantially that of space 22.

Refractory mix 36 comprises at least about 70 weight percent refractory aggregate and from about 0.5 to 20 weight percent thermosetting resin. The particulate refractory aggregate is selected from among common refractories such as deadburned magnesia, deadburned dolomite, alumina, silica, zircon and alumina-silica based, refractories. Deadburned magnesia is preferred, since it generates a minimum of inclusions in molten steel. A minimum of about 70 weight percent of the refractory aggregate is required, since below this amount the resistance of the resulting protective layer to molten steel and slag is severely reduced. At least about 90 weight percent refractory aggregate is preferred. The refractory aggregate preferably has a maximum particle size of about five millimeters; aggregates of larger size are not sufficiently free flowing to make a protective layer uniform enough to prevent penetration by the molten steel and slag.

The thermosetting resin of refractory mix 36 serves as a binder in the making of the monolithic protective layer. Any thermosetting resin may be used, such as alkyd, allylic, amino(melamine and urea), epoxy, phenolic, polyester, silicone or urethane resin, as well as combinations and modified products thereof. Phenol-formaldehyde resins have a setting temperature of from about 150 to 180°C are preferred. The resin content of the mix must be at least about 0.5 weight percent, since a lower content fails to provide a protective layer of the desired strength. The maximum resin content is about 20 weight percent, since beyond this amount of protective layer having low resistance to molten steel and slag is formed. More preferably, the resin is from about 1 to 4 weight percent of the mix. The resin may be present in the mix as a separate particulate component of the mix as long as uniform blend with the refractory aggregate is obtained. Preferably, however, the resin is coated on the refractory aggregate to insure an intimate and uniform bonding of the refractory particles.

Preferably refractory mix 36 comprises a particulate inorganic binder. The purpose of the inorganic binder is to assure a strong bond between the refractory aggregate particles in the temperature range of 500 to 800°C, for at these temperatures the resin is carbonized and loses its binding ability, with resultant easy separation of the protective layer from the working lining. The inorganic binder may be selected from among the conventional binders for refractories, such as alkali metal salts of silicic acid, for example sodium or potassium silicate; borates, for example boraic; phosphates, for example sodium hexametaphosphate, sodium tetrapolyphosphate, and sodium, potassium or ammonium monobasic phosphate. The inorganic binder is present in an amount of from about 0.5 to 10 weight percent of the mix. With inorganic binder contents less than about 0.5 weight percent, the resulting protective layer does not have the desired strength at elevated temperatures while with contents much greater than about 10 percent, the protective layer is not satisfactorily resistant to molten steel and slag and its disintegratability is low. Preferably, the inorganic binder content is from about 1 to 5 weight percent of the mix.

The refractory mix 36 preferably comprises from about 0.5 to 10 weight percent of a particulate inorganic compound having a water of crystallisation in addition to inorganic binder. Examples of such compounds include magnesium carbonate trihydrate (MgC0₃ - 3H₂0), magnesium nitrate hexahydrate (Mg(N0₃)₂ . 6H₂0), aluminum potassium sulfate dodecahydrate (AIK(SO₄)₂ · 12H₂0) and aluminum sodium sulfate dodecahydrate (AINa(SO₄)₂ · 12H₂O). The purpose of such a compound is to promote the binding effect of the inorganic binder at lower temperatures as well as to improve the effectiveness of the inorganic binder. The desired effect is negligible at contents of such compounds below about 0.5 weight percent, while with contents of such compounds above about 10 weight percent, excess released moisture from the compound causes considerable energy loss during the initial heating of the protective layer. The preferred level of such compound is from about 1 to 5 weight percent of the mix, in addition to the inorganic binder. However, if the inorganic binder already has water of crystallization as in the case of sodium silicate pentahydrate (Na2SiO3. 5H₂0), aluminum sulfate octadecahydrate (Al₂SO₄ · 18H₂0), magnesium sulfate heptahydrate (MgS0₄ . 7H₂0) and sodium tetraborate decahydrate (Na_{Z}B₄0, - 10H₂0: borax), use of additional such compound in the mix becomes unnecessary.

Refractory mix 36 may also contain up to about 10 weight percent fiber to improve the strength of the protective layer. Suitable fibers include ceramic fibers; metal fibers; carbon fibers; inorganic fibers such as rock wool, glass fibers and slag wool; and organic fibers such as cellulose and nylon. Since the fibers tend to reduce the flowability of the mix during formation of the protective layer, and also tend to make the formation of a seamless coating more difficult, the fiber length is limited to about 25 millimeters, preferably from about 5 to 15 millimeters, and the fiber content is limited to a maximum of about 10 weight percent.

The amount of compressed air used to inject refractory mix 36 into space 22 must be controlled. Enough air must be used to successfully transfer the mix from supply tank 34 to space 22 but if too much is employed, it is difficult for the air to escape from the protective layer being formed in space 22 even with many vent holes 24 in mold 16. The weight ratio of refractory mix 36 to air is therefore preferably maintained at from about 50 to 200. While air has been illustrated and is preferred, any other suitable inert gas, such as nitrogen, may be used for the transfer.

The protective layer and method of preparation of the instant invention as herein described have numerous advantages which those in the art can readily appreciate. The high disintegratability of the layer facilitates the subsequent servicing of the tundish. Since it is formed essentially dry and has superior insulating properties, requiring less energy consumption and a preheat to only about 500 to 800°C before being placed in service, the instant layer is superior to that prepared by the trowelling method. The instant layer is also superior to the lagging sheet since it is seamless and firmly secured to the working lining; in contrast to the lagging sheet, it is highly resistant to slag and molten steel and does not tend to separate from the working lining during the casting operation. Further, the instant method allows preparation of the protective layer in a fraction of the time required by either the trowelling or the lagging sheet method.

The following example is merely illustrative and is not to be construed as limiting the invention, the scope of which is defined by the claims.

### Example

A dry particulate refractory mix for the protective layer of a tundish is prepared by intimately blending in a mixer the following ingredients:

A tundish comprised of a steel shell lined with chamotte brick and with inner dimensions measuring 230 centimeters long by 60 centimeters wide by 70 centimeters deep and having two nozzles in the bottom is selected for applying a protective layer as described herein.

A mold having vent holes at various locations in its side and bottom portions is placed within the tundish with the aid of a crane such as to provide a substantially uniform space of about 30 millimeters between the outer surface of the mold and the inner surface of the tundish. The portions of the mold in contact with the nozzles and with the peripheral edge of the tundish are covered with heat resistant sealant. The refractory mix is transferred to a supply tank and the mold connected to the supply system as shown in the Figure.

Following the procedure described herein, the space between the mold and tundish is filled with about 350 kilograms of the refractory mix in about one minute, the surface of the tundish being maintained at a temperature of about 160°C during the transfer. The mold is then disconnected from the supply system, and the tundish together with the mold is transferred to a preheating zone where the mold is heated for about 5 minutes with a low flame from gas burners to heat the mold outer surface to about 180°C.

Following an additional 5-minute holding period at 160-180⁰C to cure the resin, the mold is removed from the tundish.

The tundish is then enclosed with a tundish cover, preheated to a temperature of 500 to 800°C for about 30 minutes, and immediately transferred to a casting site where continuous castings are performed. The protective layer is found to have a high resistance against the molten steel and slag, which can be easily removed from the tundish after service.

While the present invention has been described in connection with the protective layer of the tundish, those in the art can readily appreciate that it is not so limited. The present layer with its method of preparation is readily adaptable, for example, to the tundish working lining itself. In such case, the layer would be heated sufficiently to form high temperature bonding in order to give the layer the high strength required of the working lining. The method is also applicable to the linings of other vessels such as ladles, crucibles and even steelmaking vessels themselves.

## Claims

1. A method of applying a monolithic refractory layer within a metallurgical vessel, which comprises:
positioning within said vessel a mold having an outer surface substantially conforming to the configuration of the inner surface of said vessel so as to provide a substantially uniform space between said mold outer surface and said vessel inner surface;
filling said space with a substantially dry particulate mixture comprising at least about 70 weight percent refractory aggregate, from about 0.5 to 20 weight percent thermosetting resin and from about 0.5 to 10 weight percent inorganic binder;
heating said mixture to cure said resin; and removing said mold;
characterised in that either said binder has water of crystallization or said mixture comprises about 0.5 to 10 weight percent of a particulate inorganic compound having water of crystallization in addition to said binder.

2. The method of claim 1 wherein said resin is coated on said refractory aggregate.

3. The method of claim 1 or claim 2 wherein said refractory aggregate has a maximum particle size of about 5 millimetres.

4. The method of any preceding claim wherein said mixture comprises from about 1 to 5 weight percent of said particulate inorganic compound having water of crystallization in addition to inorganic binder.

5. The method of claim 4 in which said inorganic binder is sodium silicate and said particulate inorganic compound having water of crystallization is magnesium sulfate heptahydrate.

6. The method of any preceding claim wherein said mixture additionally comprises up to about 10 weight percent fiber having a length of from about 5 to 15 millimeters.

7. The method of any preceding claim 1 wherein said refractory is deadburned magnesia.

8. The method of any preceding claim wherein said resin is a phenol-formaldehyde resin and is cured at a temperature of from about 150 to 250°C.

9. The method of any preceding claim wherein said mixture is introduced to fill said space by the controlled use of pressurized gas.

10. The method of any preceding claim wherein said layer is the protective layer of a tundish.

11. The method of claim 10 wherein the thickness of said layer is from about 10 to 50 millimeters.

12. A metallurgical vessel, which comprises a monolithic layer of a resin-bonded particulate refractory aggregate applied by the method of any preceding claim.

## Patentansprüche

1. Verfahren zum Aufbringen einer monolithischen feuerfesten Schicht in einem metallurgischen Gefäß, welches umfaßt:
das Anordnen einer Form in gem genannten Gefäß, deren Außenfläche im wesentlichen der Konfiguration der Innenfläche des genannten Gefässes entspricht, um so einen im wesentlichen gleichmäßigen Raum zwischen der genannten Formaußenfläche und der genannten Gefäßinnenfläche zu bilden;
das Füllen des genannten Raums mit einer im wesentlichen trockenen Partikelmischung mit mindestens etwa 70 Gew.-% eines feuerfesten Aggregats, mit von etwa 0,5 bis 20 Gew.-% eines thermischhärtenden Harzes und mit von etwa 0,5 bis 10 Gew.-% eines anorganischen Binders;
das Erwärmen der genannten Mischung zum Aushärten des Harzes; und
das Entfernen der Form;
dadurch gekennzeichnet, daß entweder der genannte Binder Kristallwasser enthält oder die genannte Mischung etwa 0,5 bis 10 Gew.-% einer partikelförmigen anorganischen Verbindung mit Kristallwasser zusätzlich zu dem genannten Binder aufweist.

2. Verfahren nach Anspruch 1, dadurch gekennzeichnet, daß das genannten Harz auf das genannte feuerfeste Aggregat aufgezogen wird.

3. Verfahren nach Anspruch 1 oder 2, dadurch gekennzeichnet, daß das genannte feuerfeste Aggregat eine maximale Partikelgröße von etwa 5 mm besitzt.

4. Verfahren nach irgendeinem vorhergehenden Anspruch, dadurch gekennzeichnet, daß die genannte Mischung von etwa 1 bis 5 Gew.-% der genannten partikelförmigen anorganischen Verbindung mit Kristallwasser zusätzlich zu dem anorganischen Binder aufweist.

5. Verfahren nach Anspruch 4, dadurch gekennzeichnet, daß der genannte anorganische Binder Natriumsilikat ist und die genannte partikelförmige anorganische Verbindung mit Kristallwasser Magnesiumsulfatheptahydrat ist.

6. Verfahren nach irgendeinem vorhergehenden Anspruch, dadurch gekennzeichnet, daß die genannte Mischung zusätzlich bis zu etwa 10 Gew.-% Faser mit einer Länge von etwa 5 bis 15 mm enthält.

7. Verfahren nach irgendeinem vorhergehenden Anspruch, dadurch gekennzeichnet, daß das genannten feuerfeste Material totgebrannte Magnesia ist.

8. Verfahren nach irgendeinem vorhergehenden Anspruch, dadurch gekennzeichnet, daß das genannte Harz ein Phenol-Formaldehydharz ist und bei einer Temperatur von etwa 150 bis 250°C ausgehärtet wird.

9. Verfahren nach irgendeinem vorhergehenden Anspruch, dadurch gekennzeichnet, daß die genannte Mischung zum Füllen des genannten Raums durch die kontrollierte Verwendung eines Druckgases eingeführt wird.

10. Verfahren nach irgendeinem vorhergehenden Anspruch, dadurch gekennzeichnet, daß die genannte Schicht die Schutzschicht einer Gießpfanne ist.

11. Verfahren nach Anspruch 10, dadurch gekennzeichnet, daß die Dicke der genannten Schicht im Bereich von etwa 10 bis 50 mm liegt

12. Metallurgisches Gefäß, das eine monolithische Schicht aus einem harzgebundenen, partikelförmigen feuerfesten Aggregat aufweist, die mittels des Verfahrens nach irgendeinem vorhergehenden Anspruch aufgebracht ist.

## Revendications

1. Procédé pour appliquer une couche réfractaire monolithique dans un récipient métallurgique qui consiste:
à positionner à l'intérieur dudit récipient un moule ayant une surface extérieure épousant sensiblement la configuration de la surface intérieure dudit récipient afin de former un espace sensiblement uniforme entre ladite surface extérieure du moule et ladite surface intérieure du récipient;
à remplir ledit espace d'un mélange en particules sensiblement sèches comprenant au moins environ 70% en poids d'un agrégat réfractaire, environ 0,5 à 20% en poids d'une résine thermodurcissable et environ 0,5 à 10% en poids d'un liant inorganique;
à chauffer ledit mélange pour faire durcir ladite résine; et
à retirer ledit moule;
caractérisé en ce que soit ledit liant contient de l'eau de cristallisation, soit ledit mélange comprend entre environ 0,5 et 10% en poids d'un composé inorganique en particules contenant de l'eau de cristallisation, en plus dudit liant.

2. Procédé selon la revendication 1, dans lequel ledit aggrégat réfractaire est enduit de ladite résine.

3. Procédé selon la revendication 1 ou la revendication 2, dans lequel ledit agrégat réfractaire présente une dimension maximale de particules d'environ 5 mm.

4. Procédé selon l'une quelconque des revendications précédentes, dans lequel ledit mélange comprend entre environ 1 et 5% en poids dudit composé inorganique en particules contenant de l'eau de cristallisation, en plus du liant inorganique.

5. Procédé selon la revendication 4, dans lequel ledit liant inorganique est du silicate de sodium et ledit composé inorganique en particules contenant de l'eau de cristallisation est du sulfate de magnésium heptahydraté.

6. Procédé selon l'une quelconque des revendications précédentes, dans lequel ledit mélange comprend en outre jusqu'à environ 10% en poids de fibre ayant une longueur d'environ 5 à 15 mm.

7. Procédé selon la revendication 1, dans lequel ledit réfractaire est de la magnésie cuite à mort.

8. Procédé selon l'une quelconque des revendications précédentes, dans lequel ladite résine est une résine phénol-formadéhyde et est durcie à une température d'environ 150 à 250°C.

9. Procédé selon l'une quelconque des revendications précédentes, dans lequel ledit mélange est introduit pour remplir ledit espace par l'utilisation maîtrisée d'un gaz comprimé.

10. Procédé selon l'une quelconque des revendications précédentes, dans lequel ladite couche est la couche protectrice d'une panier de coulée.

11. Procédé selon la revendication 10, dans lequel l'épaisseur de ladite couche est d'environ 10 à 50 mm.

12. Récipient métallurgique, qui comprend une couche monolithique d'un aggrégat réfractaire en particules liées par une résine, appliquée par le procédé de l'une quelconque des revendications précédentes.
